

# UNITED STATES PATENT OFFICE.

FIN SPARRE, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## PYROXYLIN COMPOSITION.

1,266,073.

Specification of Letters Patent. Patented May 14, 1918.

No Drawing. Application filed September 3, 1914, Serial No. 859,972. Renewed September 28, 1917. Serial No. 193,724.

*To all whom it may concern:*

Be it known that I, FIN SPARRE, of Wilmington, in the county of New Castle, and in the State of Delaware, have invented a certain new and useful Improvement in Pyroxylin Compositions, and do hereby declare that the following is a full, clear, and exact description thereof.

My invention relates particularly to solvents used in connection with pyroxylin compositions, and the pyroxylin compositions containing the same, and my invention is applicable to the use of such compositions in connection with many different industries, although it is especially applicable for use in connection with the coating of fabrics, in the manufacture of artificial leather, patent leather, pyroxylin lacquers, etc.

The object of my invention is to provide a new solvent mixture, in which a comparatively large percentage of alcohol may be used, thereby reducing the cost of the solvent mixture, in which there is less objectionable odor than previous similar mixtures, and in which there is a rapid evaporation. A further object of my invention is to provide pyroxylin compositions containing such solvent mixtures. Other objects of my invention will appear from the discussion thereof hereinafter.

It is well known that certain grades of nitrocellulose, particularly those of relatively low nitrogen content, and nitrated under special conditions, contain a relatively large percentage of alcohol-soluble material which, when for instance ethyl alcohol of 94% by weight is used, can readily exceed 25% and may reach as high as 60% of said material and even in the case of special varieties of pyroxylin more than 70% thereof. It is also known that a mixture of ethyl alcohol and commercial benzol, for instance, of the commercial variety containing about 90% of the hydrocarbon benzene, forms an even better solvent for such varieties of nitrocellulose so that almost a complete solution of the special grades of pyroxylin may be obtained with this solvent. However, I have found that it is extremely difficult if not impossible, to obtain commercially nitrated cellulose or pyroxylin which is completely soluble in either ethyl alcohol or the

mixture of alcohol and benzol, whereas for commercial utilization of such solutions, it is frequently necessary that the solution shall be a complete one. I refer, in this connection, to such commercial uses as jellies or solutions to be used in the manufacture of artificial leather, patent leather, pyroxylin lacquers, etc.

I have also found that while a solution which is almost satisfactory with respect to the amount of the nitrocellulose dissolved and physical properties of the solution can be obtained with the use of alcohol and benzol and a special grade of pyroxylin, that the commercial application of such solution is not practical for the reason that the solution is not smooth in its flowing qualities and frequently it will deposit a precipitate on standing, while the film deposited on evaporation of the solvent does not show the desired strength.

I have found that if a relatively small percentage, say, between 3 and 10%, though a larger percentage may be used, of the total solvent, is added of a more powerful solvent such as, for instance, amyl acetate or ethyl acetate, the dissolving power of the solvent is made practically complete and the properties of the solvent become entirely satisfactory, while the film deposited is also of good quality. The principal feature of my invention is, therefore, that of bringing about the solution of nitrocellulose or pyroxylin in an alcohol-benzol solution with the assistance of a small percentage of some powerful solvent. In this particular case the nitrocellulose must be of the so-called soluble variety but the solvent combination which I have discovered does not make it necessary to use such variety of nitrocellulose as is completely soluble in alcohol and benzol and which is extremely difficult to obtain. However, all the advantages of the use of the alcohol-benzol solution are obtained such as ease and uniformity of evaporation, low specific gravity of the solution, unobjectionable odor of solution, ease of obtaining a solution of satisfactory purity and without leaving any objectionable residue due to high boiling impurities, etc. However, the addition of this small amount of more powerful solvent gives advantages over

the alcohol-benzol solution by more perfect solution and prevention of subsequent precipitation. This, for instance, may be demonstrated by taking the commercial nitro-cellulose of suitable properties and dissolving it in a mixture of alcohol and benzol which then may give a fair solution probably to the extent of dissolving 85-90% in the solvent but leaving this somewhat cloudy.

10 A fairly satisfactory solution may be obtained from this by filtering, but on standing a few days a partial precipitation is apt to take place. If, however, to this solution before the filtration, for example, 8% of 15 amyl acetate or ethyl acetate is added, it will be found that complete solution of the nitro-cellulose takes place, resulting in clarifying the solution and producing a more homogeneous and flowing product.

20 While my invention is capable of being carried out in many different ways, for the purpose of illustration I shall describe only one embodiment thereof.

A solvent mixture may be made in accordance with my invention containing forty-five to sixty per cent. of benzol, thirty to forty-five per cent. of ethyl alcohol and three to fifteen per cent. of commercial amyl acetate. In applying this in the production of 25 pyroxylin compositions, twelve per cent. of the weight of the above may be added as pyroxylin, the latter being of the variety that is at least fifty per cent. soluble in a mixture of equal parts of commercial ethyl alcohol and benzol. However, it is to be understood, of course, that the percentage of pyroxylin may be varied within wide limits according to the nature of the particular process to which the composition is 35 to be applied.

A composition of this character, as will be seen, contains a large percentage of alcohol, while at the same time a small percentage of the commercial amyl acetate may 45 be used. As a result, the composition is more economical than other similar compositions used in connection with industrial processes, and the odor is less objectionable owing to the small quantity of commercial 50 amyl acetate contained in the composition. Furthermore, the solvent mixture evaporates more rapidly.

While I have described my invention above in detail, I wish it to be understood 55 that many changes may be made therein without departing from the spirit of my invention, and that in particular, many changes may be made in the proportions of the constituents without departing from 60 my invention.

I claim:

1. A solution containing a pyroxylin, which is at least fifty per cent. soluble in a mixture of equal parts of commercial 65 ethyl alcohol and benzol, the pyroxylin be-

ing dissolved in a mixture of ethyl alcohol and benzol, together with a relatively small percentage of a more powerful solvent.

2. A solution containing a pyroxylin, which is at least fifty per cent. soluble in a mixture of equal parts of commercial ethyl alcohol and benzol, the pyroxylin being dissolved in a mixture of ethyl alcohol and benzol, together with between three and fifteen per cent. of a more powerful solvent. 70

3. A solution containing a pyroxylin, which is at least fifty per cent. soluble in a mixture of equal parts of commercial ethyl alcohol and benzol, the pyroxylin being dissolved in a mixture of ethyl alcohol and benzol, together with a relatively small percentage of amyl acetate. 80

4. A solution containing a pyroxylin, which is at least fifty per cent. soluble in a mixture of equal parts of commercial ethyl alcohol and benzol, the pyroxylin being dissolved in a mixture of ethyl alcohol and benzol, together with between three and fifteen per cent. of amyl acetate. 85

5. A composition containing pyroxylin 90 and a solvent containing forty-five to sixty per cent. benzol, thirty to forty-five per cent. alcohol and three to fifteen per cent. commercial amyl acetate.

6. A composition containing pyroxylin 95 and a solvent containing forty-five to sixty per cent. benzol, thirty to forty-five per cent. alcohol and three to fifteen per cent. commercial amyl acetate, the pyroxylin being substantially twelve per cent. of the 100 whole composition.

7. A solution containing a pyroxylin, which is at least fifty per cent. soluble in a mixture of equal parts of commercial ethyl alcohol and benzol, the pyroxylin being dissolved in a mixture of ethyl alcohol and benzol, together with a relatively small percentage of an organic acetate having a boiling point between 80° and 180° C. 105

8. A solution containing a pyroxylin, 110 which is at least fifty per cent. soluble in a mixture of equal parts of commercial ethyl alcohol and benzol, the pyroxylin being dissolved in a mixture of ethyl alcohol and benzol, together with between three and fifteen per cent. of an organic acetate having a boiling point between 80° and 180° C. 115

9. A fabric coating composition comprising a solution containing pyroxylin dissolved in a solvent mixture containing ethyl 120 alcohol, benzol and a more powerful solvent amounting to not more than 15% of the solvent mixture.

10. A fabric coating composition comprising a solution containing pyroxylin dissolved in a solvent mixture containing ethyl alcohol, benzol and a more powerful solvent 125 amounting to from 3 to 15% of the solvent mixture.

11. A fabric coating composition com- 130

prising a solution containing pyroxylin dissolved in a solvent mixture containing ethyl alcohol, benzol and amyl acetate amounting to not more than 15% of the solvent mixture.

alcohol, benzol and amyl acetate amounting to from 3 to 15% of the solvent mixture. 10

In testimony that I claim the foregoing I have hereunto set my hand.

FIN SPARRE.

Witnesses:

HAMILTON BRADSHAW,  
ROBERT J. LILLEY.

12. A fabric coating composition comprising a solution containing pyroxylin dissolved in a solvent mixture containing ethyl